

## UNITED STATES PATENT OFFICE

2,591,642

## NONDIFFUSING COLOR FORMERS COMPRISING ARYL J-ACIDS IN WHICH THE ARYL RADICAL IS PROVIDED WITH A NONDIFFUSING GROUP

Vsevolod Tulagin, Phillipsburg, N. J., and Robert F. Coles, Easton, Pa., assignors to General Aniline & Film Corporation, New York, N. Y., a corporation of Delaware

No Drawing. Application January 10, 1950,  
Serial No. 137,886

4 Claims. (Cl. 95—6)

1

The present invention relates to non-diffusing color formers of the aryl J-acid type in which the non-diffusing group appears in the aryl radical joined to the nitrogen atom in the 6-position of the J-acid, and the use of such color formers in the preparation of cyan azine dye images.

U. S. Patent 2,486,440, granted November 1, 1949, to Schmidt and Tulagin, describes the formation of azine dye images in photographic elements by developing such elements in the presence of a color former with a 2,4-diamino aniline preferably a 4,6-diamino metanilic acid. Among the color formers suggested for formation of a cyan azine dye image, there is mentioned 6-anilino-1-naphthol-3-sulfonic acid (phenyl J-acid).

The dye which is produced when using this color former has very desirable spectral characteristics. The use of the color former, however, has certain disadvantages, notably its tendency to diffuse from a silver halide emulsion when located therein. Because of this the color former when used must be employed in the developer so that a multiplicity of color development steps is inevitable.

In an effort to overcome this objection to such color former while retaining the desirable dye forming characteristics thereof and while seeking to stabilize the molecule against oxidation by photographic oxidizing agents, such as acid or alkaline ferri-cyanide bleach solutions, it was suggested that the aryl-J-acids be formulated as long alkyl chain urethanes. It was felt that such products which are described in United States Patent 2,480,815 would completely avoid the objections which manifest themselves in connection with the aryl-J-acids.

It has been found, however, that the long chain urethanes of aryl-J-acids and the corresponding carboxamides do not meet the prerequisites of the art for the reason that the urethane and the carboxamide links are rather

easily broken by dilute alkalies. The use of such non-diffusing color formers, therefore, limits the composition of the solutions employed in the processing of films by the azine method.

Considerable attention has been given to improving the azine method by supplying a color former for formation of the cyan image which partakes of the desirable characteristics of the aryl-J-acids and which are at the same time more stable than the long chain urethanes of such acids. As a result of this study, it has been discovered that color formers meeting these requirements can be produced by including a carboxyl group in the aromatic radical joined to the nitrogen atom of aryl-J-acids and utilizing such carboxylic acid group for the formation of amides designed to render the compounds fast to diffusion in silver halide emulsions and stable to dilute alkalies.

20 The preparation and use of such color formers accordingly constitute the purposes and objects of our invention.

The color formers, the preparation and use of which are contemplated herein, are represented 25 by the following structural formula:



30 in which A is a radical of aromatic character and of the benzene, naphthalene, pyridine or quinoline series, X is —CO—, —OCH<sub>2</sub>CO—, —CH<sub>2</sub>CO, or —NHCH<sub>2</sub>CO—, Y is an aliphatic radical containing a chain of at least 10 carbon atoms or an aromatic radical containing an aliphatic chain of at least 10 carbon atoms, M is hydrogen or a salt forming group, such as sodium, potassium, and the like, and R is an aliphatic hydrocarbon group having less than 4 carbon atoms.

3

Examples of compounds embraced by this formula are the following:

1.



Sodium 6-(N-acetyl-5-octadecylcarbamylmethoxy-2-naphthylamino)-1-naphthol-3-sulfonate

2.



Sodium 6-(N-acetyl-6-dodecylcarbamyl-2-naphthylamino)-1-naphthol-3-sulfonate

3.



Sodium 6-(N-acetyl-4-tetradecylcarbamylanilino)-1-naphthol-3-sulfonate

4.



Sodium 6-(N-acetyl-4-decylaminocarbamylmethyl-anilino)-1-naphthol-3-sulfonate

5.



Sodium 6-(N-acetyl-7-heptadecylcarbamyl-2-naphthylamino)-1-naphthol-3-sulfonate

6.



Sodium 6-(N-acetyl-3-heptadecylcarbamylmethylamino-anilino)-1-naphthol-3-sulfonate

7.

5



Sodium 6-(N-acetyl-2-methyl-4-octadecylcarbamyl-6-quinolylamino)-1-naphthol-3-sulfonate

10



6-[N-acetyl-4-(3-stearylaminomethyl-5-sulfo-o-tolylcarbamyl)-anilino]-1-naphthol-3-sulfonate

15



6-[N-acetyl-4-(5-carboxy-3-stearylaminomethyl-5-sulfo-o-tolylcarbamyl)-anilino]-1-naphthol-3-sulfonate

20



6-[N-acetyl-4-(5-carboxy-3-stearylaminomethyl-5-sulfo-o-tolylcarbamyl)-anilino]-1-naphthol-3-sulfonate

25



6-[N-acetyl-4-(5-carboxy-3-stearylaminomethyl-5-sulfo-o-tolylcarbamyl)-anilino]-1-naphthol-3-sulfonate

30



6-[N-acetyl-4-(5-carboxy-3-stearylaminomethyl-5-sulfo-o-tolylcarbamyl)-anilino]-1-naphthol-3-sulfonate

35



6-[N-acetyl-4-(4-sulfo-3-tridecanoyleaminophenylcarbamyl)-anilino]-1-naphthol-3-sulfonate

40



6-[N-acetyl-4-(4-sulfo-3-tridecanoyleaminophenylcarbamyl)-anilino]-1-naphthol-3-sulfonate

45



6-[N-acetyl-4-(4-sulfo-3-tridecanoyleaminophenylcarbamyl)-anilino]-1-naphthol-3-sulfonate

50



6-[N-acetyl-4-(4-sulfo-3-tridecanoyleaminophenylcarbamyl)-anilino]-1-naphthol-3-sulfonate

55



6-[N-acetyl-4-(4-sulfo-3-tridecanoyleaminophenylcarbamyl)-anilino]-1-naphthol-3-sulfonate

60



6-[N-acetyl-4-(4-sulfo-3-tridecanoyleaminophenylcarbamyl)-anilino]-1-naphthol-3-sulfonate

65



6-[N-acetyl-4-(4-sulfo-3-tridecanoyleaminophenylcarbamyl)-anilino]-1-naphthol-3-sulfonate

70



6-[N-acetyl-4-(4-sulfo-3-tridecanoyleaminophenylcarbamyl)-anilino]-1-naphthol-3-sulfonate

75



6-[N-acetyl-4-(4-sulfo-3-tridecanoyleaminophenylcarbamyl)-anilino]-1-naphthol-3-sulfonate

80



6-[N-acetyl-4-(4-sulfo-3-tridecanoyleaminophenylcarbamyl)-anilino]-1-naphthol-3-sulfonate

85



6-[N-acetyl-4-(4-sulfo-3-tridecanoyleaminophenylcarbamyl)-anilino]-1-naphthol-3-sulfonate

90



6-[N-acetyl-4-(4-sulfo-3-tridecanoyleaminophenylcarbamyl)-anilino]-1-naphthol-3-sulfonate

95



6-[N-acetyl-4-(4-sulfo-3-tridecanoyleaminophenylcarbamyl)-anilino]-1-naphthol-3-sulfonate

100



6-[N-acetyl-4-(4-sulfo-3-tridecanoyleaminophenylcarbamyl)-anilino]-1-naphthol-3-sulfonate

105



6-[N-acetyl-4-(4-sulfo-3-tridecanoyleaminophenylcarbamyl)-anilino]-1-naphthol-3-sulfonate

110



6-[N-acetyl-4-(4-sulfo-3-tridecanoyleaminophenylcarbamyl)-anilino]-1-naphthol-3-sulfonate

115



6-[N-acetyl-4-(4-sulfo-3-tridecanoyleaminophenylcarbamyl)-anilino]-1-naphthol-3-sulfonate

120



6-[N-acetyl-4-(4-sulfo-3-tridecanoyleaminophenylcarbamyl)-anilino]-1-naphthol-3-sulfonate

125



6-[N-acetyl-4-(4-sulfo-3-tridecanoyleaminophenylcarbamyl)-anilino]-1-naphthol-3-sulfonate

130



6-[N-acetyl-4-(4-sulfo-3-tridecanoyleaminophenylcarbamyl)-anilino]-1-naphthol-3-sulfonate

135



6-[N-acetyl-4-(4-sulfo-3-tridecanoyleaminophenylcarbamyl)-anilino]-1-naphthol-3-sulfonate

140



6-[N-acetyl-4-(4-sulfo-3-tridecanoyleaminophenylcarbamyl)-anilino]-1-naphthol-3-sulfonate

145



6-[N-acetyl-4-(4-sulfo-3-tridecanoyleaminophenylcarbamyl)-anilino]-1-naphthol-3-sulfonate

150



6-[N-acetyl-4-(4-sulfo-3-tridecanoyleaminophenylcarbamyl)-anilino]-1-naphthol-3-sulfonate

155



6-[N-acetyl-4-(4-sulfo-3-tridecanoyleaminophenylcarbamyl)-anilino]-1-naphthol-3-sulfonate

160



6-[N-acetyl-4-(4-sulfo-3-tridecanoyleaminophenylcarbamyl)-anilino]-1-naphthol-3-sulfonate

165



6-[N-acetyl-4-(4-sulfo-3-tridecanoyleaminophenylcarbamyl)-anilino]-1-naphthol-3-sulfonate

170



6-[N-acetyl-4-(4-sulfo-3-tridecanoyleaminophenylcarbamyl)-anilino]-1-naphthol-3-sulfonate

175



6-[N-acetyl-4-(4-sulfo-3-tridecanoyleaminophenylcarbamyl)-anilino]-1-naphthol-3-sulfonate

180



6-[N-acetyl-4-(4-sulfo-3-tridecanoyleaminophenylcarbamyl)-anilino]-1-naphthol-3-sulfonate

185



6-[N-acetyl-4-(4-sulfo-3-tridecanoyleaminophenylcarbamyl)-anilino]-1-naphthol-3-sulfonate

190



6-[N-acetyl-4-(4-sulfo-3-tridecanoyleaminophenylcarbamyl)-anilino]-1-naphthol-3-sulfonate

195





Sodium 6-[N-propionyl-4-(3-stearoylamino-5-sulfo-0-tolylcarbamylmethyl)anilino]-1-naphthol-3-sulfonate



6-(N-acetyl-5-octadecylcarbamyl-2-pyridylamino)-1-naphthol-3-sulfonic acid

The above compounds are prepared while utilizing carboxy aryl-J-acids as one of the parent materials. For this purpose there may be employed:

- 3'-carboxy-2'-naphthyl-J-acid
- 7'-carboxy-2'-naphthyl-J-acid
- 8'-carboxy-naphthoxy-2'-naphthyl-J-acid
- 7'-carboxy methoxy-2'-naphthyl-J-acid
- 4'-carboxyphenyl-J-acid
- 3'-carboxy-phenyl-J-acid
- 4'-carboxy-methylphenyl-J-acid
- 3'-carboxy methylaminophenyl-J-acid
- 2-methyl-4-carboxy-6-quinilino-J-acid
- 4-carboxy-6-pyridino-J-acid, and the like.

The amidation of these acids, however, is not as simple as is the amidation of the ordinary types of acids. Thus it is not possible to prepare the acid chlorides of the aforementioned aryl-J-acids and condense these with an amine. The preparation must be effected either (1) by forming a phosphazo compound of the desired amine and condensing this phosphazo compound with the desired aryl-J-acid, or (2) by heating with phosphorous trichloride a mixture of the desired amine and the desired aryl-J-acid suspended in pyridine. The latter reaction proceeds quite smoothly and leads to well defined products and is, therefore, the operation preferred.

The formation of amides by the reaction of a phosphazo compound and an acid is described in detail in copending application Serial No. 602,154, filed by Harry W. Grimmel et al. on June 28, 1945, and entitled "Process for the Production of Organic Amides," now Patent No. 2,508,860.

The long chain amides prepared as above are non-diffusing color formers. As such, however, they cannot be used for the preparation of multilayer color film because they are very easily oxidized and lead to the production of an overall brown stain during the normal processing of such multilayer film. It has been found necessary to convert the amides to acylamino derivatives which give the required cyan dye image on color forming development, are readily soluble in water, compatible with photographic emulsions without the production of fog or desensitization of the silver halides involved. The formation of the acylamino derivatives can be readily effected by treating the amides with the desired acid anhydride, i. e., acetic, propionic or butyric, while heating the reaction mixture.

The color formers of the present invention when dispersed in silver halide emulsion may be converted into cyan azine dye images by development with the developers of U. S. Patent No.

2,486,440, and particularly with 4- $\beta$ -hydroxy ethylamino-6-phenylamino metanilic acid. Such color formers are admirably suited for use in the processing of multilayer film by the azine method.

- 5 The developers employed in such processing contain not only the desired 2,4-diamino aniline and an alkali such as sodium carbonate, sodium hydroxide or the like, but preferably in addition the usual adjuncts such as an alkali metal bromide, i. e., potassium bromide, and an alkali metal sulfite, such as sodium sulfite. The best results accrue when there is present in the developer a coupling aid in the form of an inorganic or organic base, such as pyridine, quinoline or ammonium hydroxide.
- 10 15 The following will serve to further illustrate the invention, but it is to be understood that the same is not restricted thereto.

#### PREPARATION OF CARBOXY-ARYL-J-ACIDS

##### EXAMPLE 1

###### 6'-carboxy-2'-naphthyl J-acid

Into a 1-liter three-neck flask, equipped with an agitator and a reflux condenser were placed 25 24 g. of 6-amino-2-naphthoic acid and 225 cc. of warm water. Ammonium hydroxide (conc.) was added dropwise until a complete solution was obtained. The sodium salt of J-acid (59 g.) and neutral ammonium sulfite (150 g. at 50%) 30 and sodium metabisulfite (43 g.) were added. The mixture was refluxed for 1 $\frac{1}{4}$  hours. The sodium salt of J-acid (40 g.) was added and the mixture was refluxed for 2 hours. The hot mixture was filtered and the solid tar obtained was discarded. The filtrate was acidified with concentrated hydrochloric acid and cooled. The solid was collected by filtration and further purified by crystallization from potassium chloride solution. The material obtained was a cyan color former, giving dyes of approximately the same shade as those obtained from phenyl J-acid.

##### EXAMPLE 2

###### 7'-carboxy-2'-naphthyl J-acid

The 7'-carboxy-2'-naphthyl J-acid was obtained by the same procedure as that described for the 6'-carboxy-2'-naphthyl J-acid.

##### EXAMPLE 3

###### 8'-carboxy naphthoxy 2'-naphthyl J-acid

55 Into a 1-liter 3-neck flask, equipped with a stirrer and a reflux condenser, were placed 22 g. of 7-amino-1-naphthoxy acetic acid and 150 cc. of warm water. The mixture was stirred and treated with concentrated ammonium hydroxide solution until a complete solution had taken place. The sodium salt of J-acid (58 g.) neutral ammonium sulfite solution (100 g.) and sodium meta bisulfite (50 g.) were added in the above order and the mixture was refluxed for four hours. The resulting solution was transferred to a large beaker and acidified while still very hot with 250 cc. of concentrated hydrochloric acid. The resulting suspension was cooled and the precipitated semi-solid oil was collected by decantation. This oily precipitate was dissolved in 300 cc. of hot water and turbid solution was cleared by filtration through a layer of diatomaceous earth. The filter medium was washed with 50 cc. of water. The filtrate was treated with 250 cc. of 30% potassium chloride. The oily precipitate was collected by centrifuging, dissolved in 200 cc. of boiling water and the solution was cooled. The crystalline material so

obtained was collected by filtration, pressed as dry as possible under a rubber dam and twice washed with water. The product may be further purified by repeated crystallization from water. This material was a cyan color former which gave dyes very similar in shade to those derived from 2-naphthyl J-acid. It is well to point out that the cyan dyes derived from 2-naphthyl J-acid have less red and more green transmission than the cyan dyes derived from phenyl J-acid and are therefore more desirable.

## EXAMPLE 4

*7'-carboxy methoxy-2'-naphthyl J-acid*

The 7'-carboxy methoxy-2'-naphthyl J-acid may be prepared in essentially the same manner as described in the preceding example by substituting 7'-amino-1-naphthoxy acetic acid for the 8'-amino-1-naphthoxy acetic acid.

## EXAMPLE 5

*4'-carboxy phenyl J-acid*

Into a 3-liter 3-neck flask, equipped with a stirrer and a reflux condenser was placed a solution of 770 g. J-acid paste (54%) in 1000 cc. of water containing 95 g. of sodium hydroxide. The mixture was heated to boiling and p-amino benzoic acid (210 g.) and sodium meta bisulfite (500 g.) were added and the mixture was refluxed for 5 hours. The reaction mixture was diluted with 1000 cc. of water and acidified with concentrated hydrochloric acid to a pH of 1-2. The resulting suspension was filtered. The solid was washed repeatedly with water. The material was suspended in 3 liters of hot water and potassium acetate was added until a solution had taken place. Saturated potassium chloride solution (500 cc.) was added and the solution was cooled. The crystalline solid which had separated was collected by filtration and washed with 15% potassium chloride solution. The material was further purified by repeated crystallization from 10% potassium chloride solution. A good test for the purity of the material consists of dissolving a small portion in water and acidifying with hydrochloric acid. If the substance is pure, no precipitate will be obtained while the mixture is hot; the whole mixture will set into a jelly upon cooling.

For the preparation of non-diffusing color formers, the 4'-carboxy phenyl J-acid is best converted to the pyridine salt. This may be accomplished in the following manner:

The solid obtained above is dissolved in 2 liters of hot water containing pyridine (200 cc.). The solution is strongly acidified with concentrated hydrochloric acid and allowed to cool. The yellow crystalline solid so obtained is collected by filtration, washed with water and dried.

## EXAMPLE 6

*4'-carboxymethylphenyl-J-acid*

Into a 1-liter 3-necked flask, equipped with an agitator and a reflux condenser, were placed a solution of 10 g. of sodium hydroxide in 200 cc. of water, 66 g. of J-acid and 38 g. of p-amino phenyl acetic acid. The mixture was stirred until a solution was obtained and then 100 g. of sodium meta bisulfite was added. The resulting suspension was refluxed for 24 hours, at the end of which time all the solids had again gone into solution. The solution was acidified with concentrated hydrochloric acid (125 cc.) and the mixture was cooled. The solid so obtained was

collected by filtration and dissolved in 500 cc. of hot water. Concentrated hydrochloric acid (50 cc.) was added and the suspension so obtained was cooled to 30-40° C. The product which separated at this point was collected by filtration, washed with dilute hydrochloric acid and dried.

## EXAMPLE 7

*3'-carboxy methyl amino phenyl J-acid*

The 3'-carboxy methyl amino phenyl J-acid may be prepared by the methods given above starting with 3-aminophenyl glycine and J-acid.

## EXAMPLE 8

*2-methyl-4-carboxy-6-quinoline J-acid*

Into a 1-liter 3-necked flask, equipped with an agitator and a reflux condenser were placed 200 cc. of water, 4 g. of sodium hydroxide, 20 g. of 2-methyl-6-amino cinchoninic acid, 39 g. of J-acid and 50 g. of sodium meta bisulfite. The mixture was refluxed for one hour and treated with an additional 13 g. of J-acid. The mixture was further refluxed for an additional three hours. The resulting suspension was cooled and filtered. The solid was collected by filtration and triturated with 3 N hydrochloric acid. The insoluble material was collected by filtration and thoroughly washed with water. The solid was dissolved in hot dilute sodium hydroxide solution; the solution was acidified with acetic acid and cooled. The crystalline solid so obtained was dissolved in hot water, and the solution was strongly acidified with concentrated hydrochloric acid. The dark red solid thus obtained was collected by filtration, washed with water, and dried.

## EXAMPLE 9

*4-carboxy-6-pyridino J-acid*

The procedure is the same as in Example 8 excepting that the 2-methyl-6-amino-cinchoninic acid is replaced by an equivalent amount of 6-amino nicotinic acid.

## PREPARATION OF NON-DIFFUSING ARYL J-ACIDS

## EXAMPLE 10

A mixture of 13 g. of 5-amino-3-stearoylaminoo-p-toluenesulfonic acid and 10 g. of p-carboxyphenyl J-acid in dry C. P. pyridine (150 ml.) and dry C. P. benzene (100 ml.) is placed in a 500 ml. triple-neck flask equipped with a mechanical stirrer, dropping funnel and a reflux condenser carrying a water extractor. The mixture is heated at reflux temperature for 1 hour. The water which separates in the extractor is removed, together with a total of 100 ml. of solvents. To the stirred refluxing solution is added dropwise over a period of  $\frac{1}{2}$  hour phosphorus trichloride in dry pyridine (50 ml.). The solution is heated at reflux temperature for 3 more hours.

The solvents are removed at reduced pressure, the residue dissolved in 300 ml. of hot water, filtered, and the filtrate acidified strongly with hydrochloric acid. The solid is collected and dissolved in 500 ml. of hot water, filtered through a celite pad and the filtrate treated with 150 ml. of concentrated hydrochloric acid (or until precipitation is complete). The mixture is heated to coagulate the solid and the solid collected by filtration. The solid is extracted with 500 ml. of boiling glacial acetic acid. 20 cc. of acetic anhydride are added to the extract and the mixture is refluxed for  $\frac{1}{2}$  hour. The mixture is fil-

8

tered hot, washed with petroleum ether, and dried. The yield is 18 g. of a yellow solid. This material appears to be completely non-diffusing but is somewhat sensitive to light and should be stored in a dark bottle.

The product is 6-[N-acetyl-4-(3-stearoylamino-5-sulfo-o-tolylcarbamyl)anilino] - 1 - naphthol-3-sulfonic acid.

**EXAMPLE 11**

The procedure is the same as in Example 10 excepting that the p-carboxy phenyl J-acid is replaced by an equivalent amount of 3'-carboxy methylphenyl J-acid.

The product is 6-[N-acetyl-3-(3-stearoylamino-5-sulfo-o-tolylcarbamylmethyl) anilino]-1-naphthol-3-sulfonic acid.

**EXAMPLE 12**

The procedure is the same as in Example 10 excepting that the p-carboxy phenyl J-acid is replaced by 7'-carboxy methoxy-2'-naphthyl J-acid, and the acetic anhydride is replaced by propionic anhydride.

The product is 6-[N-propionyl-4-(3-stearoyl-amino-5-sulfo-o-tolyl-carbamylmethyl)-anilino]-1-naphthol-3-sulfonic acid.

**EXAMPLE 13**

In a 1-liter triple-necked flask equipped with a mechanical stirrer, dropping funnel and reflux condenser carrying a water extractor and heated on a metal bath is placed a mixture of 104 g. of 3-amino-4-octadecylamino-benzene sulfonic acid pyridine salt and 88 g. of the pyridine salt of *p*-carboxyphenyl J-acid and 300 ml. of dry pyridine and 200 ml. of dry benzene. The mixture is heated at reflux and any water that collects on the separator is taken off. After the removal of water is substantially complete, a total of 250 ml. of solvents will be removed by the extractor. Phosphorus trichloride (13.7 g.) in dry benzene (50 ml.) is added rapidly dropwise. After the addition is complete, the solvents are removed as rapidly as possible by distillation. The heating is continued until a sample when removed and treated with about 1 ml. of glacial acetic acid and 5 ml. of acetic anhydride and boiled for one minute and then cooled produces a well-defined crystalline product. The reaction mixture is then treated with 200 ml. of glacial acetic acid and 500 ml. of acetic anhydride and heated for 10 minutes. The solution is then diluted with 300 ml. additional of acetic anhydride and cooled. The solid is collected, sucked as dry as possible on the funnel and washed with acetic anhydride and then acetone. The product may be purified from crystallization from 50% mixture of glacial acetic acid and absolute alcohol. It is presumably the pyridine salt of 6-[N-acetyl-4-(2-octadecyl-acetamido-5-sulfo-phenylcarbamyl)anilino]-1-naphthol-3-sulfonic acid, or of 6-*p*-[4-(1-octadecyl-5-sulfo-2-benzimidazolyl)phenylcarbamyl]-N-acetylanilino-1-naphthol-3-sulfonic acid.

**EXAMPLE 14**

In a 500 ml. triple-necked flask equipped with a mechanical stirrer, dropping funnel and reflux condenser carrying a water separator and heated on a metal bath is placed a mixture of 52 g. of the pyridine salt of 3-amino-4-octadecylamino benzene sulfonic acid and 36 g. of m-carboxy-phenyl J-acid in 150 ml. of dry pyridine and 100 ml. of dry benzene. The mixture is dried in a manner similar to the above example. A solu-

10

tion of phosphorus trichloride (6.9 g.) and benzene (50 ml.) is added dropwise with stirring at reflux. After the addition is complete, the solvents are removed by distillation and the heating of the residue is continued for one hour. The resulting syrup is treated with acetic acid to obtain a solution which is diluted with acetone and the precipitated solvent is collected. The solid is refluxed with absolute ethanol and lithium carbonate and the resulting solution filtered and cooled. Low boiling petroleum ether is added to precipitate the lithium salt. The lithium salt is dissolved in a mixture of glacial acetic acid and acetic anhydride and the mixture refluxed for  $\frac{1}{2}$  hour to form the N-acetylamino derivative. The solution is cooled and the precipitated salt is collected by filtration.

The product is 6-[N-acetyl-3-(2-octadecylamino-5-sulfophenylcarbamyl)anilino]-1-naphthol-3-sulfonic acid.

**EXAMPLE 15**

To a solution of 54 g. of octadecylamine and 32 g. of triethylamine in 200 cc. of anhydrous toluene kept at 60°–80° C. is added slowly a solution of 14 g. of phosphorus trichloride in 35 cc. of anhydrous toluene and the whole is refluxed for two and one-half hours. The precipitated triethylamine hydrochloride is removed by filtration and the phosphazone solution (the filtrate) so obtained is used without further purification.

35 A mixture of 10.5 g. of potassium 6-[8'-(carboxymethoxy)-2'-naphthyl] amino-1-naphthol-3-sulfonate and 250 cc. of anhydrous xylene is refluxed under a water separator until no more water can be detected in the reflux. The phosphazo solution prepared according to the above (80 cc.) is added and the mixture is kept at 110-125° for 20 hours. Acetic acid (8 cc.) is added  
40 and the mixture is refluxed for ½ hour. A solution of 10 g. of potassium acetate in 25 cc. of glacial acetic acid is added and the mixture is refluxed for ½ hour. Acetic anhydride (20 cc.) is added and the mixture is refluxed for ½ hour.  
45 The resulting suspension was evaporated at reduced pressure. The residue was thoroughly extracted by refluxing with 250 cc. of absolute alcohol. The mixture was cooled and the yellow solid product was collected by filtration. This  
50 substance is a non-diffusing cyan color former of the probable constitution:

6 - N - acetyl-8-octadecylcarbamylmethoxy-2-naphthylamino)-1-naphthol-3-sulfonic acid.



It can be further freed from residual phosphorus compounds by boiling with aqueous sodium carbonate solution, acidifying and precipitating with the aid of brine.

**EXAMPLE 16**

The procedure is the same as in Example 15 excepting that the aryl J-acid thereof is replaced by an equivalent amount of 2-methyl-4-carboxy-6-quinolino J-acid.

The product is 6-(N-acetyl-2-methyl-4-octadecylcarbamyl-6-quinolylamino)-1-naphthol-3-sulfonic acid.

## 11

USE OF NON-DIFFUSING COLOR FORMERS  
IN SILVER HALIDE EMULSIONS

## EXAMPLE 17

A photographic silver bromide emulsion containing per kilo of emulsion 1.5 gram of the color former of Example 10 is exposed, the latent image developed in a Metol-hydroquinone developer, re-exposed, and the residual silver halide developed for 10 minutes in a solution of the following composition:

|                                                              |                   |      |
|--------------------------------------------------------------|-------------------|------|
| Potassium carbonate                                          | grams             | 20   |
| Sodium sulfite                                               | do                | 60   |
| Ethylene diamine                                             | cubic centimeters | 30   |
| 4-( $\beta$ -hydroxyethylamino)-6-phenylamino-metanilic acid | grams             | 3    |
| Water                                                        | cubic centimeters | 1000 |

The developed silver images are bleached with potassium ferricyanide and fixed in an acid hardening hypo solution. There is thus obtained a cyan dyestuff image which is stable to acids and alkali oxidizing agents.

## EXAMPLE 18

An integral tripack having as the bottom layer a red sensitive emulsion containing as the cyan color former the product of Example 13, as the middle layer a green sensitive emulsion containing as the magenta color former 2-stearoyl-amino-6-(8'-hydroxy cinchinoylamino)-toluene-4-sulfonic acid, and as the outermost layer a blue sensitive emulsion containing as the yellow color former 2-(benzoylacetamidophenyl)-1-octadecyl-5-benzimidazole sulfonic acid, was exposed, developed in black and white, re-exposed and the residual silver halide developed for 12 minutes in a developer of the following composition:

|                                                              |                   |      |
|--------------------------------------------------------------|-------------------|------|
| 6-phenylamino-4-( $\beta$ -hydroxyethylamino)-metanilic acid | grams             | 8    |
| Potassium carbonate                                          | do                | 20   |
| Sodium sulfite                                               | do                | 60   |
| Potassium bromide                                            | do                | 10   |
| Benzylamine                                                  | do                | 5    |
| Water to                                                     | cubic centimeters | 1000 |

The film after development is washed, bleached in a ferricyanide bleach, and fixed in an acid hardening hypo. There was thus obtained a positive dyestuff image in each of the three layers—a cyan dye image in the bottom layer, a magenta dye image in the middle layer, and a brilliant yellow dye image in the top layer.

It is to be understood that any of the color formers referred to above may be dispersed in silver halide emulsions and employed for the production of azine dye images.

Various modifications of the invention will occur to operators in this field, and we accordingly do not intend to be limited in the patent granted except as necessitated by the appended claims.

We claim:

1. A photographic silver halide emulsion containing as a color former fast to diffusion a compound of the following constitution:



wherein A is a radical of aromatic character selected from the class consisting of those of the benzene, naphthalene, pyridine and quinoline series, X is a carbonyl containing group selected from the class consisting of those of the following formulae: —CO—, —OCH<sub>2</sub>CO—, —CH<sub>2</sub>CO—, and —NHCH<sub>2</sub>CO—, Y is a radical selected from the class consisting of those of aliphatic radicals containing a chain of at least 10 carbon atoms and aromatic radicals containing an aliphatic chain of at least 10 carbon atoms, M is selected from the class consisting of hydrogen and salt forming groups, and R is an aliphatic hydrocarbon group having less than 4 carbon atoms.

## 12

selected from the class consisting of those of the benzene, naphthalene, pyridine and quinoline series, X is a carbonyl containing group selected from the class consisting of those of the following formulae: —CO—, —OCH<sub>2</sub>CO—, —CH<sub>2</sub>CO—, and —NHCH<sub>2</sub>CO—, Y is a radical selected from the class consisting of those of aliphatic radicals containing a chain of at least 10 carbon atoms and aromatic radicals containing an aliphatic chain of at least 10 carbon atoms, M is selected from the class consisting of hydrogen and salt forming groups, and R is an aliphatic hydrocarbon group having less than 4 carbon atoms.

2. The process of producing an azine dye image which comprises developing with a 2,4-diamino-aniline, an exposed silver halide emulsion containing as a color former, a compound of the following formula:



wherein A is a radical of aromatic character selected from the class consisting of those of the benzene, naphthalene, pyridine and quinoline series, X is a carbonyl containing group selected from the class consisting of those of the following formulae: —CO—, —OCH<sub>2</sub>CO—, —CH<sub>2</sub>CO—, and —NHCH<sub>2</sub>CO—, Y is a radical selected from the class consisting of those of aliphatic radicals containing a chain of at least 10 carbon atoms and aromatic radicals containing an aliphatic chain of at least 10 carbon atoms, and M is selected from the class consisting of hydrogen and salt forming groups.

3. A photographic silver halide emulsion containing as a color former fast to diffusion a compound of the following formula:



4. The process of producing a cyan azine dye image which comprises developing with a 2,4-diamino aniline an exposed silver halide emulsion containing as a color former fast to diffusion a product of the following formula:



VSEVOLOD TULAGIN.  
ROBERT F. COLES.

## REFERENCES CITED

The following references are of record in the file of this patent:

## UNITED STATES PATENTS

| 70 | Number    | Name     | Date          |
|----|-----------|----------|---------------|
|    | 2,186,849 | Wilmanns | Jan. 9, 1940  |
|    | 2,480,815 | Tulagin  | Aug. 30, 1949 |